



US005508582A

# United States Patent [19]

Sugimoto et al.

[11] Patent Number: 5,508,582

[45] Date of Patent: Apr. 16, 1996

[54] SPARK PLUG INSULATOR FOR USE IN INTERNAL COMBUSTION ENGINE

5,283,134 2/1994 Sugimoto et al. .... 313/143

[75] Inventors: Makoto Sugimoto; Masahiro Konishi; Hiroyuki Tanabe; Kenichi Nishikawa, all of Nagoya, Japan

## FOREIGN PATENT DOCUMENTS

|         |        |                    |
|---------|--------|--------------------|
| 0544952 | 6/1993 | European Pat. Off. |
| 2207474 | 8/1990 | Japan.             |
| 4098783 | 3/1992 | Japan.             |

[73] Assignee: NGK Spark Plug Co., Ltd., Nagoya, Japan

Primary Examiner—Donald J. Yusko

Assistant Examiner—Nimesh D. Patel

Attorney, Agent, or Firm—Sughrue, Mion, Zinn, Macpeak &amp; Seas

[21] Appl. No.: 231,836

[22] Filed: Apr. 25, 1994

## [57] ABSTRACT

## [30] Foreign Application Priority Data

Apr. 26, 1993 [JP] Japan ..... 5-099206

[51] Int. Cl. 6 H01T 13/38; H01T 21/02

[52] U.S. Cl. 313/118; 313/123; 313/143

[58] Field of Search 313/118, 123, 313/143

In a spark plug insulator for use in an internal combustion engine, a sintered body has boron nitride and a metal oxide, the boron nitride of the sintered body being 80% or greater by weight, and the sintered body having a thermal expansion coefficient of less than  $5.0 \times 10^{-6}/^{\circ}\text{C}$ . The metal oxide is selected alone or in combination from the group consisting of magnesium oxide, calcium oxide, silicon oxide, boron oxide, yttrium oxide and aluminum oxide.

## [56] References Cited

## U.S. PATENT DOCUMENTS

4,970,095 11/1990 Bolt et al. ..... 427/226

2 Claims, 3 Drawing Sheets



Fig. 1



Fig. 2



Fig. 3



## SPARK PLUG INSULATOR FOR USE IN INTERNAL COMBUSTION ENGINE

### BACKGROUND OF THE INVENTION

#### 1. Field of the Invention

This invention relates to a spark plug insulator of an internal combustion engine and a method of making the same for use in an automobile and aircraft, and particularly a spark plug insulator which is improved to be superior in insulation and thermal-shock resistance.

#### 2. Description of Prior Art

In an internal combustion engine, a spark plug insulator is exposed to the ambient temperature as high as 2000° C. at an explosion stroke, and then exposed to an air-fuel mixture which has a temperature equivalent to the atmosphere at an intake stroke. This causes the insulator to be alternately subjected to a heat-and-cool cycle repeatedly so as to give the insulator repetitive thermal stress. This type of insulator has been made from a sintered ceramic material with aluminum oxide (alumina) as a main component.

With the recent demand of a high output with a high fuel efficiency of the internal combustion engine, it has been increasingly difficult to cope with an enhanced temperature of the combustion gas which causes a thermal shock on the insulator made of the aluminum oxide based ceramic material. It is found that the thermal shock finally induces cracks on the insulator made of the aluminum oxide based ceramic material depending on bench test conditions.

Therefore, it is an object of the invention to provide a spark plug insulator which is capable of improving a thermal-shock resistance due to repetitive thermal stress so as to prevent cracks on the insulator.

### SUMMARY OF THE INVENTION

According to the invention, there is provided a spark plug insulator comprising a sintered body including boron nitride and a metal oxide, the boron nitride of the sintered body being 80% or greater by weight, and the sintered body having a thermal expansion coefficient of less than  $5.0 \times 10^{-6}/^{\circ}\text{C}$ .

According further to the invention, there is provided a spark plug insulator wherein a component of the metal oxide is less than 20% by weight, and is selected alone or in combination from the group consisting of magnesium oxide, calcium oxide, silicon oxide, boron oxide, yttrium oxide and aluminum oxide.

According to the invention, there is also provided a method of making a spark plug insulator comprising steps of: mixing a powder of boron nitride (BN), an additive and ethanol to form a mixture within a nylon pot mill by means of a nylon ball, the boron nitride being 80% or greater by weight; drying the mixture for about 10 hours in a vacuum environment; pulverizing the dried mixture so that its grain size is less than 350  $\mu\text{m}$ ; forcing the pulverized mixture into a tubular carbon die; sintering the mixture in the carbon die by means of hot press in a nitrogen atmosphere under about 50 MPa at 1800°~1900° C. for 5~10 hours so as to form a boron nitride based compact body; and releasing the boron nitride based compact body from the carbon die.

With the use of the sintered body made of the boron oxide based ceramic which is superior in thermal-shock resistance to the alumina based insulator, it is possible to effectively cope with the increased temperature of the combustion gas

which is caused from the recent demand of the high fuel efficiency of the internal combustion engine.

When the component of the boron nitride is less than 80% by weight, an increased dependency on other additives except boron oxide sacrifices the thermal-shock resistance characteristic of the boron nitride based insulator. When the thermal expansion coefficient of the boron nitride based insulator exceeds  $5.0 \times 10^{-6}/^{\circ}\text{C}$ , its thermal-shock resistance substantially reduces to that of the alumina based insulator, thus losing its advantages over the alumina based insulator.

With an additive of the metal oxide selected alone or in combination from the group consisting of magnesium oxide, calcium oxide, silicon oxide, boron oxide, yttrium oxide and aluminum oxide, it is possible to provide the boron nitride based insulator with a high insulation property.

When the component of the metal oxide exceeds 20% by weight, boron nitride is decomposed to increase unfavorable voids in the sintered body during the process in which boron nitride reacts with the metal oxide to form nitrogen oxide gas.

These and other objects and advantages of the invention will be apparent upon reference to the following specification, attendant claims and drawings.

### BRIEF DESCRIPTION OF THE DRAWINGS

FIG. 1 is a plan view a spark plug according to a first embodiment of the invention, with its left half being shown in section;

FIG. 2 is a flow chart showing a process how a spark plug insulator is manufactured; and

FIG. 3 is a plan view a spark plug according to a second embodiment of the invention, with its left half being shown section.

### DETAILED DESCRIPTION OF THE EMBODIMENT OF THE INVENTION

Referring to FIG. 1 which shows a spark plug 1 used for an automobile and aircraft engine, the spark plug 1 has a metallic shell 2, L-shaped ground electrode 3, center electrode 4 and tubular insulator 5. The metallic shell 2 forms an outer structure of the spark plug 1, and works as a tool for securing the spark plug to the engine and supporting the insulator 5. An upper end of the metallic shell 2 forms a hexagonal portion 6 which is used for applying a wrench or the like. A lower end of the metallic shell 2 forms a male thread 7 which is attached to a cylinder head of the engine. To the lower end surface of the metallic shell 2, the Ground electrode 3 is secured by means of welding or the like. The electrodes 3, 4 are heat and erosion resistant material made of Ni—Cr—Fe based alloy or Ni—Mn—Si based alloy due to the fact that they are exposed to the high temperature environment of the combustion gas in a combustion chamber of the engine. A spark Gap G is provided between a firing end of the ground electrode 3 and a front end of the center electrode 4. A noise-suppressive resistor 10 is disposed between a middle axis 9 of a terminal electrode 8 and the center electrode 4 which the insulator 5 holds within its bore 51. The center electrode 4 is axially aligned by melting a conductive glass sealing powder 11 between the center electrode 4 and the resistor 10 and between the resistor 10 and the middle axis 9. The insulator 5 is supported within the metallic shell 2 by caulking its rear end 2a. Integrally with the insulator 5, a leg portion 13 is made at the side which is exposed to the high temperature environment of the combustion gas in a combustion chamber of the engine. With the rear end of the insulator 5, a corrugated portion 14 is integrally provided in which the middle axis 9 of the

terminal electrode **8** is enclosed.

The insulator **5** is a sintered body made of boron nitride (BN) and a metal oxide superior in insulation. A component of the boron nitride (BN) is 80% or more by weight, and a component of the metal oxide is less than 20% by weight. The boron nitride based insulator **5** has a thermal expansion coefficient less than  $5.0 \times 10^{-6}/^{\circ}\text{C}$ . The metal oxide is selected alone or in combination from the group consisting of magnesium oxide (MgO), calcium oxide (CaO), silicon oxide (SiO<sub>2</sub>), boron oxide (B<sub>2</sub>O<sub>3</sub>), yttrium oxide (Y<sub>2</sub>O<sub>3</sub>) and aluminum oxide (Al<sub>2</sub>O<sub>3</sub>).

In making the insulator **5**, we employ powder of 99.0% pure boron nitride (BN) (1  $\mu\text{m}$  in average grain size) including ceramic materials consisting of 0.90% B<sub>2</sub>O<sub>3</sub>, 0.02% CaO or the like as impurity substances. As an additive to the powder of the boron nitride (BN), we use MgO, CaO (converted to CaCO<sub>3</sub>), SiO<sub>2</sub>, B<sub>2</sub>O<sub>3</sub>, Al<sub>2</sub>O<sub>3</sub>, Y<sub>2</sub>O<sub>3</sub>, TiO<sub>2</sub> and ZrO<sub>2</sub> alone or in combination as described hereinafter in specimens 1-7 at Table 1. Each of the additive is 99.0% pure, and having an average grain size of less than 1  $\mu\text{m}$ .

The specimens of the insulator **5** are manufactured as follows:

The powder of the boron nitride (BN), the additive and ethanol are mixed together to form a mixture within a nylon pot mill by means of a nylon ball (mixing process in FIG. 2).

Then, the mixture is dried for 10 hours in a vacuum environment (desiccant process in FIG. 2). Thereafter, the dried mixture is pulverized so that its grain size is less than 350  $\mu\text{m}$  (pulverization process in FIG. 2). The pulverized mixture is forced into a tubular carbon die which measures 25 mm in diameter and 100 mm in length. The mixture in the carbon die is sintered by means of hot press in a nitrided oxygen atmosphere under 50 MPa at 1800°-1900° C. for 5-10 hours (sintering process in FIG. 2). The mixture, having undergone the sintering process, forms a boron nitride based compact body (specimens 1-7 and counterparts 1-5 at Table 1).

Then, the boron nitride based compact body is separated from the carbon die (releasing process). A tiny amount of the compact body is taken out to analyze its components. In the analyzing process, an oxygen component is detected by means of an infrared gas analysis, and CaO, Y<sub>2</sub>O<sub>3</sub>, Al<sub>2</sub>O<sub>3</sub>, MgO or the like are analyzed by means of fluorescent X-ray analysis. By measuring an amount of oxygen component remained after allotting it to the metal oxides, B<sub>2</sub>O<sub>3</sub> is calculated. The boron nitride (BN) is determined by deducting the metal oxides from the total weight. In each of the specimens, an ignorable amount of carbon is perceived, and therefore, the amount of the carbon is not shown in Table 1.

The boron nitride based compact body is shaped into the insulator **5** which is suitable for the spark plug **1** (finishing process). After the center electrode **4** is inserted into the insulator **5**, the conductive glass sealing powder **11** and the resistor **10** are inserted into the insulator **5**. The middle portion of the insulator **5** is heated at 900°-1000° C., and at the same time, the terminal electrode **8** is press fit into the insulator **5** to seal the connection between the rear end of the center electrode **4** and the axis **9**. The insulator **5** is placed within the metallic shell **2**, to the front end **2b** of which the ground electrode **3** is welded (assembling process).

Physical properties of the specimens and the counterparts are compared on the basis of experimental test result shown in Tables 1 and 2.

Table 1 shows the boron nitride (wt %), the additive (wt %), sintering conditions, relative density (%) and appearance of voids in the insulator **5** for the spark plug **1** (specimens 1-7 and counterparts 1-5).

Table 2 shows an engine and measurement test result of a thermal expansion coefficient (°C.), insulation (MΩ) and thermal-shock resistance (°C.) in the insulator **5** for the spark plug **1** (specimens 1-7 and counterparts 1, 4 and 5). In the counterpart **6**, the corresponding physical properties are measured in an alumina-based insulator for a spark plug.

TABLE 1

| No.                | boron nitride<br>(BN) (%) | additive<br>(%)                                                              | sintering conditions |      | relative density<br>(%) | note                                |
|--------------------|---------------------------|------------------------------------------------------------------------------|----------------------|------|-------------------------|-------------------------------------|
|                    |                           |                                                                              | (°C.)                | (hr) |                         |                                     |
| <u>specimen</u>    |                           |                                                                              |                      |      |                         |                                     |
| 1                  | 81.1                      | CaO: 14.3<br>B <sub>2</sub> O <sub>3</sub> : 4.6                             | 1850                 | 5    | 97                      |                                     |
| 2                  | 90.1                      | Y <sub>2</sub> O <sub>3</sub> : 7.8<br>MgO: 2.1                              | 1900                 | 5    | 98                      |                                     |
| 3                  | 94.8                      | TiO <sub>2</sub> : 3.9<br>B <sub>2</sub> O <sub>3</sub> : 1.3                | 1900                 | 10   | 98                      |                                     |
| 4                  | 98.9                      | B <sub>2</sub> O <sub>3</sub> : 1.1                                          | 1900                 | 10   | 98                      |                                     |
| 5                  | 98.5                      | CaO: 1.5                                                                     | 1900                 | 10   | 98                      |                                     |
| 6                  | 99.5                      | B <sub>2</sub> O <sub>3</sub> : 0.5                                          | 1900                 | 10   | 98                      |                                     |
| 7                  | 93.5                      | SiO <sub>2</sub> : 5.5<br>Al <sub>2</sub> O <sub>3</sub> : 1.0               | 1850                 | 10   | 97                      |                                     |
| <u>counterpart</u> |                           |                                                                              |                      |      |                         |                                     |
| 1                  | 76.6                      | CaO: 5.2<br>Al <sub>2</sub> O <sub>3</sub> : 18.2                            | 1800                 | 10   | 96                      | increased<br>appearance<br>of voids |
| 2                  | 60.0                      | Y <sub>2</sub> O <sub>3</sub> : 9.7<br>Al <sub>2</sub> O <sub>3</sub> : 30.3 | 1800                 | 10   | 92                      | increased<br>appearance<br>of voids |
| 3                  | 49.9                      | SiO <sub>2</sub> : 18.9<br>Al <sub>2</sub> O <sub>3</sub> : 31.2             | 1800                 | 10   | 90                      | increased<br>appearance<br>of voids |
| 4                  | 81.2                      | ZrO <sub>2</sub> : 14.7<br>Al <sub>2</sub> O <sub>3</sub> : 4.1              | 1850                 | 10   | 95                      |                                     |
| 5                  | 69.1                      | SiO <sub>2</sub> : 9.6<br>Al <sub>2</sub> O <sub>3</sub> : 21.3              | 1800                 | 5    | 94                      |                                     |

TABLE 2

| No.                | thermal<br>expansion<br>coefficient<br>( $^{\circ}\text{C.}$ ) | insulation<br>( $\text{M}\Omega$ ) | thermal shock<br>resistance ( $^{\circ}\text{C.}$ ) | engine<br>test |
|--------------------|----------------------------------------------------------------|------------------------------------|-----------------------------------------------------|----------------|
| <u>specimen</u>    |                                                                |                                    |                                                     |                |
| 1                  | $4.1 \times 10^{-6}$                                           | 1000                               | 380                                                 | good           |
| 2                  | $2.4 \times 10^{-6}$                                           | 1800                               | 650                                                 | good           |
| 3                  | $3.8 \times 10^{-6}$                                           | 20                                 | 800                                                 | misfire        |
| 4                  | $1.2 \times 10^{-6}$                                           | >10000                             | >1000                                               | good           |
| 5                  | $1.8 \times 10^{-6}$                                           | 9500                               | 1000                                                | good           |
| 6                  | $1.5 \times 10^{-6}$                                           | >10000                             | >1000                                               | good           |
| 7                  | $2.0 \times 10^{-6}$                                           | 800                                | 700                                                 | good           |
| <u>counterpart</u> |                                                                |                                    |                                                     |                |
| 1                  | $3.2 \times 10^{-6}$                                           | 1200                               | 280                                                 | no good        |
| 4                  | $6.0 \times 10^{-6}$                                           | 200                                | 280                                                 | no good        |
| 5                  | $4.6 \times 10^{-6}$                                           | 250                                | 230                                                 | no good        |
| 6                  | $7.8 \times 10^{-6}$                                           | 600                                | 200                                                 | no good        |

The relative density (%) in Table 1 is estimated by (apparent density)/(calculated density). The structural observation of the insulator specimens is carried out by using SEM (Scanning Type Electronic Microscope). The thermal expansion coefficient of the insulator specimens is measured between  $25^{\circ}\text{C}$ . (room temperature) and  $1000^{\circ}\text{C}$ . in the nitrogen atmosphere by using a push-pull type thermal expansion meter.

With the use of an insulation resistor meter (at 1000 V), the insulation is estimated by measuring the resistance between the ground electrode and the terminal electrode, while at the same time, heating the specimens at 500 in the nitrogen atmosphere.

The thermal-shock resistance is estimated on the basis of a difference between the water temperature ( $20^{\circ}\text{C.}$ ) and each temperature of the specimens in which cracks occur by shaping the specimens 1~7 and the counterparts 1, 4, 5 and 6 into an elongation ( $\phi 20 \text{ mm} \times 20 \text{ mm}$ ) which are respectively dipped into water after taking them out of a heated furnace ( $180^{\circ}\text{--}1000^{\circ}\text{C.}$ ).

An experimental engine test is carried out with the specimens mounted on a four-cycle, single cylinder engine. With the passage of five minutes after a heated portion 12 of the insulator reaches the temperature in which preignition occurs, it is investigated whether or not cracks occur on the specimens 1~7 and the counterparts 1, 4, 5 and 6. Depending on whether or not the cracks occur, the engine condition is represented by good or no-good as shown in Table 2.

As apparently confirmed from the above investigation, an increased appearance of voids is observed in the texture of the counterparts 1~3 since they contain the boron nitride (BN) in less than 80% by weight. In particular, it is found that the specimens 1 and 5 are inferior in thermal-shock

resistance on which the cracks occur in the experimental engine test.

The counterpart 4 has a thermal expansion coefficient of  $6.0 \times 10^{-6}/^{\circ}\text{C.}$  which is greater than that of the specimens 1~7. This causes cracks in the experimental engine test although the counterpart 4, which has the boron nitride of more than 80% by weight, is superior in thermal-shock resistance to the counterpart 6.

The specimen 3 is as low as 20  $\text{M}\Omega$  in insulation property due to the addition of  $\text{TiO}_2$ , and induces a misfire by electrical leakage when starting the engine.

As evident from the foregoing description, it is possible to obtain an insulator superior in thermal-shock resistance to the alumina based insulator by using the sintered body made of the boron nitride based ceramic being 80% or more by weight, and the metal oxide less than 20% by weight with its thermal expansion coefficient less than  $5.0 \times 10^{-6}/^{\circ}\text{C.}$  This makes it possible to substantially improve the thermal-shock resistance caused from the repetitive thermal stress so as to effectively cope with the increased temperature of the combustion gas which is caused from the recent demand of the high fuel efficiency of the internal combustion engine.

FIG. 3 shows a second embodiment of the invention in which a two-part type insulator 15 is placed in the metallic shell 2 of the spark plug 1. The two-part type insulator 15 includes the leg portion 13 and an alumina-based ceramic body 17 secured to the leg portion 13 by means of mortise-tenon joint. The leg portion 13 is made of a boron nitride based ceramic body 16, and positioned at the side of the heated portion 12. A rear end of the alumina-based ceramic body 17 has a corrugated portion 14. In the second embodiment of the invention, it is cost-effective particularly when putting the spark plug insulator into mass production by providing the leg portion 13 with the boron nitride based ceramic body 16.

While the invention has been described with reference to the specific embodiments, it is understood that this description is not to be construed in a limiting sense in as much as various modifications and additions to the specific embodiments may be made by skilled artisans without departing from the spirit and scope of the invention.

What is claimed is:

1. A spark plug insulator comprising a sintered body including boron nitride and a metal oxide, the boron nitride of the sintered body being at least 80% by weight, and the sintered body having a thermal expansion coefficient of less than  $5.0 \times 10^{-6}/^{\circ}\text{C.}$

2. A spark plug insulator as recited in claim 1, wherein the metal oxide is less than 20% by weight, and is selected alone or in combination from the group consisting of magnesium oxide, calcium oxide, silicon oxide, boron oxide, yttrium oxide and aluminum oxide.

\* \* \* \* \*